

## UNITED STATES PATENT OFFICE

2,399,096

## PRODUCTION OF MAGNESIUM-CONTAINING MIXTURES

Alva C. Byrns, Oakland, Calif., assignor, by mesne assignments, to The Permanente Metals Corporation, a corporation of Delaware

No Drawing. Application February 21, 1944,  
Serial No. 523,361

11 Claims. (Cl. 75—4)

This invention relates to a method for preparing a magnesium-containing mixture, particularly a mixture to be used for the preparation of magnesium metal by reduction.

A number of methods have been devised for recovering magnesium from its ores or from compounds containing magnesium and there are included in these methods reduction processes wherein materials containing magnesium in combination with oxygen are reduced to yield the free metal. One of these processes, known in the art as the carbothermic process, comprises the reduction of a magnesium-oxygen compound with a carbonaceous reducing agent, yielding entirely gaseous products of reaction from which the magnesium is condensed and recovered.

The method of producing the mixture of the magnesium compound and the carbonaceous reducing agent has been the subject of considerable investigation. It has been known to mix finely ground or powdered magnesia, or other source of magnesium, with finely ground or powdered solid carbonaceous material such as coke, charcoal, graphite. In an attempt to obtain more intimate admixture of the magnesium compound and the reducing agent it has also been known to add a binding agent, such as tar, pitch, tar oil, asphalt or the like to the primary mixture of ore, or other compound, and the coke or charcoal. This binder has then been carbonized prior to reduction. It has been considered preferable to form the mixture into briquets and then to carbonize the binder. This is believed to be a more effective way of holding the magnesia, for example, and the carbonaceous reducing agent in intimate contact in the heated zone during the reducing operation.

It is a two-fold object in preparing carbothermic feed to get the magnesium compound and the carbonaceous reducing agent into intimate contact, one with the other, and to maintain this intimate contact as, for instance, by making the mixture into a briquet which will be strong and stable under handling or heating. It has been found in practice that mixtures or briquets made as described above have had less than the desired strength and stability and the components have tended to burst apart upon heating, as when rapidly heated to the temperatures required for reduction. This has led to incomplete reaction and decreased yield of the desired magnesium metal. Particles of small size, which break off, are carried out of the furnace before reaction takes place, for example, and thus significant amounts of unreacted MgO and reducing agent are carried over with the effluent vapors from the reaction zone.

I have now found that the aforesaid objects can be attained and the above disadvantages overcome by admixing finely divided magnesium

compound with a liquefiable, thermoplastic carbonaceous reducing agent and then subjecting to destructive distillation to form a carbonized or preferably a coked, matrix having the magnesium compound dispersed therethru.

In one method of practicing my invention, the magnesium compound, such as magnesia, magnesium hydroxide, magnesite, brucite, basic carbonate or the like is suitably made into a dispersion or suspension in a liquefiable carbonaceous material such as bituminous or coking coal, bitumens, tar, pitch, residual fuel oil, crude petroleum, heavy petroleum residue, cracked petroleum residue, molasses or the like, or mixtures of such materials. This suspension or dispersion is then heated to cause coking or carbonization, without attaining conditions under which the magnesium compound would be reduced. The coked mass may then be broken up into pieces of suitable size and used directly, or it may be ground and formed into the desired agglomerate, using a binder, for example, tar, pitch, or the like, if necessary. However, pellets may be formed by the use of pressure alone if high enough pressures are employed. Alternatively, briquets, pellets, nodules or other shapes may be formed of the magnesium compound—liquefiable, thermoplastic hydrocarbon mixture and these formed pieces then coked. It is found in practical operations that formed pieces are more conveniently handled both before and during reduction.

The mixtures of reactants formed as described above react smoothly, uniformly and quickly in the reducing zone and excel in these characteristics over the furnace feeds produced according to former methods. This is shown more clearly by the examples in the table below, wherein the term "furnace feed" is used to describe a feed made by combining MgO and petroleum coke, both finely divided, with a binder of coal tar pitch and baking to carbonize the binder. The "fuel oil and MgO coke" describes a feed made by coking a mixture of a fuel oil which was a heavy liquid hydrocarbon having a density of 45 13.4° A. P. I. and finely divided MgO with stirring to prevent segregation. These tests were carried out in a small induction furnace and "Kw." represents the input in kilowatts. Helium was passed through the furnace, to maintain an inert atmosphere, at the rate of 2½ liters per minute.

| Feed                   | Pellet No.            | Pellet weight, grams | Temp. of reaction, °C. | Kw. | Sublimation time in minutes |
|------------------------|-----------------------|----------------------|------------------------|-----|-----------------------------|
| 55 Furnace feed...     | Average of 6 pellets. | 0.6163               | 1940                   | 8.9 | 9.13                        |
| Fuel oil and MgO coke. | Average of 4 pellets. | .6513                | 1894                   | 8.4 | 7.25                        |

By visual observation thru a sight-hole in the induction furnace it is evident that the start of reaction is slower with the "furnace feed" than with the fuel oil-MgO coke, that the reaction is then quite rapid in the case of the furnace feed, after which it slows down to the end, and that the reaction with the fuel oil-MgO coke, in contrast, is smooth and uniform. The table above is an example of the speedier over-all reaction with the latter material.

It is believed that these advantages are derived from the circumstances that the carbonaceous materials of my invention become plastic upon heating and flow about, over and around and in the interstices between the fine MgO particles and are carbonized in stronger and more intimate contact with the MgO particles than has heretofore been possible. By my invention, it is believed that there is produced a continuous phase of carbon having finely divided MgO dispersed therethru and that the carbon is formed adhering to the surface of the MgO particle, so that it forms a sort of a jacket for the small MgO particle. Such firm contact makes it possible for reaction to proceed even after the jacketed MgO particle may have split off from the main briquet, or other, mass. Processes which have hitherto been known have produced a binding phase of coke containing particles of MgO and also discrete particles of the coke or carbon originally added as the reducing agent. My process avoids the presence of these discrete carbon particles and produces a strongly bonded mixture wherein the surface to surface forces act between the MgO particles and the continuous carbon phase. The mixture obtained by my process has a uniformly black appearance and, even when finely subdivided, as by thorough grinding, no light-colored magnesium compound particles are evident. This is true even upon microscopic examination.

As a specific example of the method of preparing the magnesium-containing mixture having a content of carbonaceous reducing material, I place 800 gallons of 13.4° A. P. I. fuel oil (6523 lbs.) in a tank equipped with a paddle agitator and circulating pump, and add thereto 3025 lbs. of finely ground MgO. The whole is thoroughly mixed to give a uniform suspension and is then transferred to the coking zone. This zone is a shell still suitable for carrying out destructive distillation of the heavy fuel oil and is, in this instance, a horizontal drum, externally fired, equipped for circulation of the oil-MgO mixture by pumping out of the bottom of the drum at one end and back into the drum at the other end. The still is also provided with a vapor exit line, and with a suitable condenser, and collector for the condensate, as well as an exit line for non-condensable gases. The still is also fitted with an inlet for sweeping gases.

The oil mixture is introduced into the heated drum and heating continued while the oil mixture is circulated to cause agitation and prevent settling out of the MgO. Circulation is continued until the oil becomes so viscous that pumping is difficult and at this stage it is viscous enough to hold the MgO in suspension. Distillation is continued for 22.5 hours or until the production of condensate has practically ceased. Natural gas is now admitted to the drum to sweep out residual heavy vapors and these are collected by way of the condenser and condensate collector also.

There are obtained 4050 lbs. of MgO-coke mixture and 669 gals. (5024 lbs.) of distillate. The

coke mixture shows a content of 21.4% fixed carbon and 73.9% of ash, principally MgO. The solid coked mass is broken up into pieces of suitable size for charging to the reduction furnace.

When other liquefiable, thermoplastic carbonaceous materials are employed in my process, variations in the above procedure can be practiced. In the case of quite fluid materials, mixers can be installed in the coking zone to maintain agitation and prevent segregation of the magnesium compound. Where the carbonaceous material is solid or sufficiently viscous, as for instance in the case of suitable coal or high melting point pitch, the components of the mix can be finely divided, thoroughly mixed, and heated to coke with little or no agitation.

Pitch, however, foams upon heating and tends to produce a final coked product having a very spongy appearance. This may be desirable in some cases but where it is not desired, it is advantageous to prepare the coking mixture by admixing a proportion of a fuel oil or heavy petroleum residue to reduce this tendency and to produce a denser, uniformly coked final mass. As an example of this procedure, I mix together 437 parts by weight of fuel oil, 85 parts by weight of a coal tar pitch having a melting point of about 330° F., and 478 parts by weight of magnesia. 987 parts by weight of this mixture are destructively distilled by heating to 1030° F. over a period of 90 minutes, with mechanical agitation for about half this time. The distillate recovered amounts to 342 parts by weight. The coke mixture obtained contains 19.5% of fixed carbon. A quite dense final mass can also advantageously be obtained by coking MgO with a liquid hydrocarbon having a proportion of powdered coking coal admixed therewith.

Other inert gases may be used to sweep the residual heavy, vaporizable materials out of the coking drum at the end of the distillation. Other types of coking stills may of course be used. In coking a mixture of low viscosity, for example, the mixture may be partially distilled in one zone as by the recirculation by pumping as described, for instance, and the partially distilled mixture then transferred to another piece of equipment, such as a coking oven or other device, for final coking.

The condensate collected is useful in a number of ways, or it may be fractionated to recover components having specific desired boiling point ranges, or the like.

Alternatively, in making the coked mixture, segregation may be prevented by mixing MgO which has been heated to a high temperature, for example to incandescence, with pitch, petroleum residue or other suitable carbonaceous material. The components may be mixed by spraying simultaneously into a heated tower or in any other desired way. Immediate, intimate contact between incandescent MgO and the reducing agents described, in this manner, causes very rapid carbonization and produces good distribution.

The mixture prepared may be used in carbothermic reduction processes described above or in other processes, such as a process for preparing MgCl<sub>2</sub> by treatment in the presence of chlorine. When used in the carbothermic process for making magnesium, however, there are a number of specific advantages. It is noted that the metal content of the condensate from this process is higher by about 5% than that heretofore obtainable. The reduction furnace is found to operate smoothly at lower temperatures with consequent

reduction in crucible erosion and improvement in operation of the electrode glands. Due to more efficient reaction with less development of free carbon in the reaction mass there is less arcing in the reaction bed and less dissipation of the metallurgical coke therein, having the result that it is not necessary to feed in as much of such coke as formerly.

In order to make a dense, hard and highly reactive product it is advantageous in some cases to add a relatively small proportion of the coked mixture, finely ground, to the starting material. For instance, I may admix about 5% to 10% of coked MgO-fuel oil fines to a starting mixture of MgO and fuel oil, and coke the mass to obtain a very hard, dense coke mass. This mass also contains the magnesium compound in firm and intimate contact with the reducing agent and shows increased strength and increased reactivity. The table below indicates the increase in reactivity.

| Feed                                 | Pellet No. | Pellet weight, grams | Temp. of reaction, °C. | Kw.  | Sublimation time in minutes |
|--------------------------------------|------------|----------------------|------------------------|------|-----------------------------|
| Furnace feed.....                    | 9          | 5.50                 | 1955-2000              | 11.5 | 20                          |
| Fuel oil, MgO, and fines, coked..... | 4          | 5.60                 | 1970-2010              | 11.5 | 15                          |

It is to be understood that the above detailed description has been given for the purpose of illustration and that modifications and variations can be made therein without departing from the spirit and scope of the appended claims.

Having now described my invention what I wish to claim is:

1. Process for preparing a magnesium-containing mixture which comprises uniformly dispersing a magnesium compound in a liquefiable, thermoplastic carbonaceous material containing substantially no non-coking solid carbonaceous material, and heating to destructively distil said carbonaceous material whereby there is produced a continuous carbon phase having the magnesium compound dispersed therethrough.

2. Process for preparing a magnesium-containing mixture for the recovery of Mg by reduction of an oxide compound thereof which comprises uniformly dispersing a magnesium oxide compound in a liquefiable, thermoplastic carbonaceous reducing agent containing substantially no non-coking solid carbonaceous material, and heating to coke said reducing agent.

3. Process for preparing a magnesium-containing mixture for the recovery of magnesium by reduction of an oxide thereof which comprises uniformly dispersing a finely divided magnesium oxide and finely divided coking coal in a heavy liquid hydrocarbon containing substantially no non-coking solid carbonaceous material, and coking said coal and said hydrocarbon with agitation during the first part of the distillation period, whereby there is produced a continuous carbon phase having finely divided MgO dispersed therethrough.

4. Process for preparing a magnesium-containing mixture for the recovery of magnesium by reduction of an oxide thereof comprising uniformly dispersing magnesium oxide in a heavy liquid hydrocarbon containing substantially no non-coking solid carbonaceous material, destructively distilling said hydrocarbon with agitation during the first part of the distillation, and recovering a coked mass containing said magnesium oxide in dispersion in a continuous carbon phase.

5. Process for preparing a magnesium-containing mixture for the recovery of magnesium by reduction of an oxide thereof comprising uniformly mixing finely divided MgO and finely divided high melting point pitch containing substantially no non-coking solid carbonaceous material, and heating said mixture to recover a coked mass comprising a continuous carbon phase having finely divided MgO dispersed therethrough.
- 10 6. Process for preparing a magnesium-containing mixture for the recovery of magnesium by reduction of an oxide thereof which comprises preparing an intimate mixture of finely divided MgO, finely divided high melting point pitch and heavy liquid hydrocarbon, said mixture containing substantially no non-coking solid carbonaceous material and destructively distilling said mixture with agitation during the first part of the distillation to recover a coked mass.
- 15 7. Process for preparing a magnesium-containing mixture for the recovery of magnesium by reduction of an oxide thereof which comprises preparing a uniform suspension of MgO in heavy liquid hydrocarbon containing substantially no non-coking solid carbonaceous material, heating with agitation to partially destructively distil said hydrocarbon, then continuing heating without agitation to complete said distillation, and recovering a coked mass.
- 20 8. Process for preparing a magnesium-containing mixture which comprises preparing an intimate mixture of a liquefiable, thermoplastic carbonaceous agent and MgO said mixture containing substantially no non-coking solid carbonaceous material, heating to obtain a coked mass, finely dividing said coked mass, preparing a second intimate mixture containing a liquefiable, thermoplastic carbonaceous agent, MgO and said finely divided coked mass, and heating to coke said second intimate mixture.
- 25 9. Process for preparing a magnesium-containing mixture which comprises preparing an intimate mixture of a liquefiable, thermoplastic carbonaceous agent and MgO, said mixture containing substantially no non-coking solid carbonaceous material, heating to obtain a coked mass, grinding said coked mass, admixing a binder therewith, forming agglomerates of said coked mass and binder, and heating to coke the binder.
- 30 10. Process for preparing a magnesium-containing mixture which includes preparing an intimate mixture of a liquefiable, thermoplastic carbonaceous agent and MgO, said mixture containing substantially no non-coking solid carbonaceous material, heating to destructively distil said carbonaceous agent, recovering a coked mass containing said MgO, and separately condensing and recovering the distillate from said carbonaceous agent.
- 35 11. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 40 12. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 45 13. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 50 14. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 55 15. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 60 16. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 65 17. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.
- 70 18. Process for preparing a magnesium-containing mixture which comprises preparing a uniform suspension of MgO in fuel oil containing substantially no non-coked solid carbonaceous material, heating to partially destructively distil while recirculating to maintain said MgO in suspension, continuing heating to completely destructively distil, recovering a coked mass containing said MgO dispersed therethru, and separately condensing and recovering the distillates from said destructive distillations, the said destructive distillations being carried out with the introduction of a current of inert gas.

ALVA C. BYRNS.